



US005811229A

# United States Patent [19]

**Van den Zegel****[11] Patent Number: 5,811,229****[45] Date of Patent: Sep. 22, 1998**

[54] **RADIOGRAPHIC IMAGE FORMING FILM-SCREEN SYSTEM WITH BLUE PIGMENT**

[75] Inventor: **Marc Van den Zegel**, Boortmeerbeek, Belgium

[73] Assignee: **AGFA-Gevaert, N.V.**, Mortsel, Belgium

[21] Appl. No.: **787,379**

[22] Filed: **Jan. 22, 1997**

[30] **Foreign Application Priority Data**

Feb. 19, 1996 [EP] European Pat. Off. .... 96200417

[51] **Int. Cl.<sup>6</sup>** ..... **G03C 1/825**; G03C 5/17

[52] **U.S. Cl.** ..... **430/517**; 430/139; 430/502; 430/965; 430/966

[58] **Field of Search** ..... 430/139, 502, 430/517, 966, 965

[56] **References Cited**

U.S. PATENT DOCUMENTS

3,705,807 12/1972 Busatto ..... 430/517  
4,900,652 2/1990 Dickerson et al. ..... 430/966  
5,213,951 5/1993 Delfino et al. ..... 430/966

5,252,443 10/1993 Dickerson ..... 430/966  
5,468,599 11/1995 Biavasco et al. ..... 430/966

*Primary Examiner*—Richard L. Schilling  
*Attorney, Agent, or Firm*—Breiner & Breiner

[57]

## ABSTRACT

An image-forming film-screen system for medical diagnostic imaging is disclosed comprising a light-sensitive silver halide photographic film material in operative association with at least one intensifying screen comprising on a support a layer of a visible light emitting luminescent phosphor, the said film material comprising a support and on at least one side thereof a light-sensitive silver halide emulsion layer having spectrally sensitized tabular silver halide and a non-light-sensitive protective layer, wherein said protective layer contains a polymeric compound selected from the group consisting of gelatin, a synthetic, semi-synthetic or natural substitute for gelatin and latex (co)polymers, in an amount of at least 0.4 g per m<sup>2</sup>; characterized in that between a light-sensitive silver halide emulsion layer and said protective layer there is an intermediate layer comprising a blue colored pigment in dispersed form, having a solubility in isopropanol at 25° C. of less than 10 mg per liter.

**10 Claims, No Drawings**

## RADIOGRAPHIC IMAGE FORMING FILM-SCREEN SYSTEM WITH BLUE PIGMENT

### DESCRIPTION

#### Field of the Invention

This invention relates to a radiographic image forming screen-film system of at least one intensifying screen and a light-sensitive silver halide photographic material in operative association therewith.

#### Background of the Invention

In radiology classical screen-film systems still remain important. In a screen-film system phosphors present in an intensifying screen convert X-ray radiation into visible light. The photons of visible light emitted from said phosphors are then absorbed by adjacent radiographic film material containing light-sensitive silver halide emulsion crystals.

For applications, such as mammography and diagnosis of extremities, where radiographic images having high sharpness are required, suitable screen-film systems usually contain only one screen. Light-sensitive silver halide photographic layer(s) coated at only one side of a film support are used in this application, wherein the outermost layer of said film should be in close contact with the said screen in favour of sharpness.

For general applications wherein a higher sensitivity is preferred red the screen-film system contains two screens. Between the said screens the film is positioned and comprises on each side of the support at least one light-sensitive silver halide photographic layer.

In the said light-sensitive layer tabular silver halide emulsion crystals are frequently used nowadays. Tabular grains are disclosed e.g. in U.S. Pat. No. 4,414,304 for their high covering power and developability and in U.S. Pat. Nos. 4,425,425 and 4,425,426 for their lower cross-over. All these effects are the result of a higher surface to volume ratio characteristic for said tabular grains.

Said higher surface to volume ratio also provides adsorption of higher amounts of spectral sensitizing dyes, offering the advantage of absorption of more incident light, thereby reducing cross-over.

One disadvantage however resulting from the presence of higher amounts of spectral sensitizing dye(s) is dye stain after processing, due to incomplete removal of said dye(s) from the processed material.

Another unacceptable disadvantage of tabular grains is the yellow-brown color of the developed silver after processing, especially when said grains have a thickness of less than 0.30  $\mu\text{m}$ . For thinner tabular grains even a more tremendous deterioration from the desired black image tone is observed, especially when the image is examined in transparency as well as under reflected light conditions.

A solution for these problems has been described in e.g. EP-A 0 468 211 and in EP-A 0 655 645. Therein a blue colored pigment is added to the photographic sensitive layer or another layer of the film in order to reduce residual dye stain and to provide a black image tone. This blue pigment is characterized by an absorption maximum of from 570 to 630 nm and from 640 to 700 nm respectively. In the examples of EP-A's 0 468 211 and 0 655 645 this pigment is added to the light-sensitive emulsion layer containing silver halide emulsion crystals. Due to the presence of huge amounts of spectral sensitizers adsorbed at the large surface area of the tabular silver halide emulsion grains, dye stain is

a serious problem, and, as has been established in EP-A 0 468 211, the presence of said blue pigment reduces the amount of water soluble iodide and bromide salts necessary to get formation of J-aggregates of the spectral sensitizers used in favour of reducing cross-over. As has further been described in that application the pigment must be insoluble in water and at least be insoluble in the solvent in which the pigments are used.

However the presence of a blue pigment in a photographic element in operative association with an intensifying screen enhances the risk of staining of the surface of said screen so that artefacts can occur on the image formed after contact with such stained screen. This phenomenon especially occurs after cleaning the screen surface with solvents used as screen-cleaners. As a consequence of frequent cleaning procedures it often happens that a stained screen is obtained that cannot be cleaned anymore.

Moreover blue pigment escaping from the film material often makes dirty the rollers in the automatic processing machine wherein the exposed film material is processed, thereby disturbing images generated on the following films processed therein.

#### Objects and Summary of the Invention

Therefore it is an object of the present invention to prevent staining of intensifying screens during exposure when used in operative association with radiographic film materials comprising blue pigments, incorporated therein to prevent dye staining by spectral sensitizers adsorbed at the surface of tabular silver halide emulsion grains present in light-sensitive emulsion layers of said film materials and/or to improve blackness of images (developed silver) resulting from developed tabular grains.

It is a further object of this invention to prevent staining of the rollers in automatic processing machines during processing said exposed materials. Other objects of this invention will become apparent from the description hereinafter.

Therefore an image-forming film-screen system for medical diagnostic imaging is disclosed comprising a light-sensitive silver halide photographic film material in operative association with at least one intensifying screen comprising on a support a layer of a visible light-emitting luminescent phosphor, the said film material comprising a support and on at least one side thereof a light-sensitive silver halide emulsion layer having spectrally sensitized tabular silver halide and a non-light-sensitive protective layer, wherein said protective layer contains a polymeric compound selected from the group consisting of gelatin, a synthetic, semi-synthetic or natural substitute for gelatin and latex (co)polymers, in an amount of at least 0.4 g per  $\text{m}^2$ ; characterized in that between a light-sensitive silver halide emulsion layer and said protective layer there is an intermediate layer comprising a blue colored pigment in dispersed form, having a solubility in isopropanol at 25° C. of less than 10 mg per liter.

#### Detailed Description of the Invention

The best results to improve the color of silver generated from developed tabular silver halide grains present in light-sensitive layers of exposed radiographic film material used in the screen-film system according to this invention are obtained when the blue dye or pigment is present in an intermediate layer located between a light-sensitive silver halide emulsion layer situated farther than any other silver halide emulsion layer, if present, from the film support and

a non-light-sensitive protective layer of a photographic material. Said protective layer corresponds with the protective antistress layer, whereupon in some applications an afterlayer may be coated.

It is necessary to use blue dyes having low solubility in isopropanol, in order to prevent dye staining of said screens. Isopropanol is normally used as a screen cleaner.

It is important that in this invention at least said protective antistress layer and, if present, said afterlayer, contains a polymeric compound in an amount of at least 0.2 g per m<sup>2</sup> and more preferably at least 0.4 g/m<sup>2</sup>. Said protective antistress layer may be composed of two different layers, the layer more close to the support acting as an intermediate layer comprising said blue dye(s) in dispersed form. Said two different layers may have the same composition, except for the presence of said blue dye(s) in dispersed form.

In order to provide a film material applicable in rapid processing applications it is further important to have said polymeric compound in an amount of not more than 2 g/m<sup>2</sup>, especially with regard to drying velocity.

According to this invention said polymeric compound is a compound selected from the group consisting of gelatin, a synthetic, semi-synthetic or natural substitute for gelatin, and latex (co)polymers. The presence of (additional) amounts of (natural or synthetic) clay and/or colloidal silica is further highly appreciated in favor of physical surface characteristics as such as glare, slidability, etc.

Gelatin is well-known as an essential polymeric compound of hydrophilic colloid layers in photographic materials. Synthetic substitutes for gelatin are e.g. polyvinyl alcohol, poly-N-vinyl pyrrolidone, polyvinyl imidazole, polyvinyl pyrazole, polyacrylamide, polyacrylic acid, and derivatives thereof, in particular copolymers thereof. Natural substitutes for gelatin are e.g. other proteins such as zein, albumin and casein, cellulose, saccharides, starch, and alginates. In general, the semi-synthetic substitutes for gelatin are modified natural products e.g. gelatin derivatives obtained by conversion of gelatin with alkylating or acylating agents or by grafting of polymerizable monomers on gelatin, and cellulose derivatives such as hydroxyalkyl cellulose, carboxymethyl cellulose, phthaloyl cellulose, and cellulose sulphates.

Gelatin can be lime-treated or acid-treated gelatin. The preparation of such gelatin types has been described in e.g. "The Science and Technology of Gelatin", edited by A. G. Ward and A. Courts, Academic Press 1977, page 295 and next pages. The gelatin can also be an enzyme-treated gelatin as described in Bull. Soc. Sci. Phot. Japan, No. 16, page 30 (1966).

Examples of said latex (co)polymers used in the film material used in the film-screen system according to this invention have been described in e.g. Research Disclosure 19551, Jul. 1980, in EP-A's 0 452 568; 0 534 006; 0 558 196 and 0 643 326; in U.S. Pat. Nos. 3,443,946; 3,589,908; 3,640,721; 4,476,218 and 4,810,624 and in JP-A 06 250 315. Especially preferred latex polymers are e.g. latex polymers comprising polyacrylic acid as described in JP-A 05 134 336 and in EP-A 0 644 456.

Clays set forth hereinbefore are disclosed e.g. in EP-A 0 644 454, wherein i.a. particular synthetic clays have been described, which are very suitable to reach good surface characteristics.

In a preferred embodiment colloidal silica as disclosed in e.g. EP-A 0 670 517 is added to the coating solution(s) of the protective antistress layer and/or to an afterlayer, if present.

In another embodiment gelatin-grafted polymer particles as disclosed e.g. in U.S. Pat. Nos. 5,393,650 and 5,426,020

or matte polymeric particles covalently bound to gelatin and colloidal silica as disclosed in U.S. Pat. No. 5,300,411 are added to the coating solution(s) of the protective antistress layer and/or to an afterlayer, if present. Said polymeric

matting particles may be covered by a layer of colloidal inorganic particles as described in e.g. in U.S. Pat. Nos. 5,288,598 and 5,378,577. Organic polymer particles as described in e.g. U.S. Pat. Nos. 4,914,012 and 5,342,733 may also be added as well as matting agents described in e.g. JP-A 04 162 032. Lubricants may further be added as described e.g. in U.S. Pat. No. 4,766,059 and in JP-A 05 107 687.

In a preferred embodiment of this invention said blue colored pigment present in dispersed form in an intermediate layer between emulsion layer and protective layer has a maximum absorption in the visible wavelength region from 570 to 700 nm and more preferred in the visible wavelength region from 570 to 630 nm as especially green-emitting screens are preferred in the film-screen system according to this invention in favour of reduced cross-over and sharpness.

Preferred blue colored dyes are selected from the group consisting of phthalocyanine dyes and indanthrone dyes as illustrated in the Examples hereinafter. It is clear that a mixture of blue colored pigments can be used, the proviso that at least one of these pigments has a maximum absorption in the visible range of the wave-length spectrum from 570 to 700 nm, and more preferred in the range from 570 to 630 nm, and that the solubility of said dyes is less than 10 mg per liter in isopropanol at 25° C. In principle pigments or dyes having a maximum absorption for said wavelength values fulfilling the solubility conditions set forth hereinbefore can additionally be added to the coating layers of the material as e.g. magenta colored dyes for use as "color correcting dyes".

According to this invention said blue pigment(s) is (are) present in an intermediate layer coated between an emulsion layer situated farther from the film support than any other emulsion layer, if present, and a protective antistress layer in an amount of from 1 mg/m<sup>2</sup> to 100 mg/m<sup>2</sup>, and more preferably in an amount of from 1 mg/m<sup>2</sup> to 50 mg/m<sup>2</sup>.

Said blue pigments are preferably dispersed by the methods described e.g. in EP-A 0 569 074 and in EP-Application No. 95202034, filed Jul. 24, 1995. Further dispersion techniques which may be applied have been described in e.g. EP-A's 0 552 646 and 0 595 821 and in U.S. Pat. No. 4,900,652. Preferred mean particle sizes of the dispersed pigments are not more than 2  $\mu$ m, more preferably not more than 1  $\mu$ m and most preferably not more than 0.5  $\mu$ m.

By making use of said selected blue colored pigment(s) in the prescribed amounts in the intermediate layer or interlayer coated upon the emulsion layer farthest from the support, a solution is offered for the problems situated hereinbefore: a suitable black image tone is obtained for the processed spectrally sensitized silver halide tabular grains and there is no staining of the intensifying phosphor screens after making frequent contact with films comprising said blue colored pigments, even not after a cleaning procedure wherein organic solvents are used, particularly isopropanol. No staining is further observed on the rollers of automatic processing machines wherein said films are run after exposure.

According to this invention light-sensitive spectrally sensitized tabular silver halide grains are used in at least one emulsion layer, wherein said tabular grains have an aspect ratio of from 2 to 20, a thickness from 0.06 to 0.30  $\mu$ m, more preferably from 0.08 to 0.22  $\mu$ m and wherein said grains

account for at least 50%, more preferably at least 70% and even more preferably at least 90% of the total projective area of all grains. In a more preferred embodiment aspect ratios of said tabular grains are from 5 to 20 and the said thickness of the grains is varying from 0.08 to 0.25  $\mu\text{m}$ . A preferred variation coefficient of less than 0.30, more preferred less than 0.20 and still even more preferred from 0.10 to 0.15 is highly appreciated. Such low variation coefficient can be attained by application of methods described in e.g. U.S. Pat. Nos. 5,147,772; 5,147,773; 5,171,659; 5,210,013 and 5,215,879.

Silver halide compositions of said tabular grains can be silver bromide, silver bromoiodide, silver chloride, silver chlorobromide, silver chloroiodide or silver chlorobromoiodide. Halide ions may be divided homogeneously or heterogeneously over the grain volume, dependent on the preparation method used. Preparation methods for tabular grain emulsions have been described e.g. in EP-A 0 569 075 (in a gelatinous dispersing medium), in EP-A 0 677 773 (in colloidal silica) and in Research Disclosures 22534, January 1983; 232012, August 1983 and 36544, September 1994, i.a. in part I (Emulsion grains and their preparation). Coated amounts of silver in the silver halide emulsion layer(s) of the film material used in the system according to this invention are in the range from 2 to 6  $\text{g/m}^2$ , and more preferably, from 3 to 5  $\text{g/m}^2$  and per side, expressed as an equivalent amount of silver nitrate.

Vehicles, vehicle extenders, vehicle-like addenda and vehicle related addenda which may be used in the context of this invention can be found in the same RD 36544, part II. Washing procedures for said emulsions can be applied as described in part III of the said RD. Emulsions coated in the film material used in the system according to this invention may be chemically sensitized as described in RD 36544, chapter IV.

According to this invention said light-sensitive tabular silver halide grains are spectrally sensitized to the blue or to the green region of the wavelength spectrum, the green region however being preferred. Spectral sensitizers used therefor have been described in RD 22534, January 1983, in RD 36544, chapter V, in EP-Application No. 95202096, filed Aug. 1, 1995, in EP-A's 0 752 034, 0 712 036, 0 712 034, 0 105 425, 0 144 091, 0 300 382, 0 487 010, 0 677 773 and 0 678 772 and in U.S. Pat. Nos. 4,942,121 and 5,108,887.

Development acceleration in order to enhance speed in the same processing cycle or in order to maintain speed in a shorter developing time can be accomplished by incorporating in the emulsion layer or adjacent layers various compounds, preferably polyoxyalkylene derivatives having a molecular weight of at least 400 such as those described in e.g. U.S. Pat. Nos. 3,038,805; 4,038,075 and 4,292,400 or development accelerators described in EP-A's 0 634 688 and 0 674 215.

UV absorbing dyes, optical brighteners and luminescent dyes can be used as described in RD 36544, chapter VI. Antifoggants and stabilizers can be used as described in the same RD, chapter VII. In Chapter VII of the said RD i.a. useful absorbing dyes, used as antihalation dyes are summarized. Further useful filter dyes have been described e.g. in EP-A's 0 656 401 and 0 724 191 and in EP-Application No. 93001438, filed Dec. 22, 1993.

Coating physical property modifying addenda like coating aids, plasticizers, lubricants, antistats and matting agents useful in the preparation of the coating solutions of the light-sensitive and non-light sensitive film layers are further described in RD 36544, chapter IX.

The gelatin binder of the radiographic film materials used in the system according to the present invention can be hardened with appropriate hardening agents such as those of the epoxide type, those of the ethylenimine type, those of the vinylsulfone type e.g. 1,3-vinylsulphonyl-2-propanol or di(vinylsulphonyl)-methane, ethylene di(vinyl-sulphone), vinylsulphonyl-ether compounds and vinylsulphonyl compounds having soluble groups, aldehydes like e.g. formaldehyde, glyoxal, and glutaric aldehyde, N-methylol compounds e.g. dimethylolurea and methyloldimethylhydantoin, dioxan derivatives e.g. 2,3-dihydroxy-dioxan, active vinyl compounds e.g. 1,3,5-triacyloyl-hexahydro-s-triazine, active halogen compounds e.g. 2,4-dichloro-6-hydroxy-s-triazine, and mucohalogenic acids e.g. mucochloric acid and mucophenoxychloric acid. These hardeners can be used alone or in combination. The binder can also be hardened with fast-reacting hardeners such as carbamoylpyridinium salts as disclosed in U.S. Pat. No. 4,063,952 and with the onium compounds as disclosed in EP-A 0 408 143. In order to get sufficiently hardened the binder should dispose of an acceptably high number of functional groups, which by reaction with an appropriate hardening agent can provide a sufficiently resistant layer. Such functional groups are especially amino groups, but also carboxylic groups, hydroxy groups, and active methylene groups.

In order to get a film material applicable in rapid processing applications it is necessary to have a film material that has been hardened to such an extent that a water absorption per gram of gelatin is not more than 3 g per gram of gelatin and even more preferred a water absorption of not more than 2 g per gram of gelatin. Said amount of water absorption is determined after incubating a sample of said film material at 57° C. and 34% RH for 3 days, weighing said sample, immersing it in distilled water at 21° C. for 3 minutes, squeezing it in order to get a surface free from water drops and weighing it again. Calculation of the differences in weight, divided by the surface area of the film strip and by the amount of gelatin coated per square meter gives the required value.

Another more suitable way to express the requirement to sufficiently harden the binder in the film material used in the screen-film system of this invention is to express it as a procentual swelling degree: the said procentual swelling degree, should not exceed a value of 300%, and more preferably should not exceed a value of 200%. Therefore after incubating a sample of a material at 57° C. and 34% RH for 3 days the thickness (a) of the layer assemblage is measured. Thereafter the sample is immersed in distilled water at 21° C. for 3 minutes and the thickness (b) of the swollen layer is measured.

The swelling ratio is then calculated as:

$$\frac{(b-a)}{a} \times 100 (\%)$$

Layers and layer arrangements which can be applied to the film material in the system according to this invention are those described in EP-A's 0 752 617, 0 712 036, 0 712 034, 0 677 773, 0 678 772, 0 610 608; 0 610 609 and in EP-A 0 569 075, in U.S. Pat. Nos. 4,092,168 and 4,311,787; in DE 2,453,217 and in GB Patent 7,907,440.

Supports and subbing layers coated adjacent thereto, useful for the film materials in the system according to this invention, can be those as described in RD 36544, chapter XV, polyethylene naphthalate inclusive. For high speed processing applications a useful subbing layer is disclosed e.g. in JP-A 01 166 031. Vinylidene chloride and styrene-

butadiene copolymers are the most well-known polymers for practical use as subbing layer ingredient in the film material of the screen-film system of this invention. Antistatic agents can be provided therein as e.g. in U.S. Pat. No. 5,391,472.

According to this invention a preferred screen in the screen-film system according to this invention is an intensifying screen comprising a green light-emitting luminescent phosphor, and more preferred a  $\text{Gd}_2\text{O}_2\text{S}:\text{Tb}$  luminescent phosphor.

In the system according to this invention a screen or a combination of screens can be used as has been described e.g. in EP-A's 0 592 724, 0 510 754, 0 647 258 and 0 648 254.

For double side coated film materials used in the system according to this invention it is clear that any combination of a symmetrical or asymmetrical film arrangement together with a symmetrical or asymmetrical pair of screens is useful. Herein the term "symmetrical or asymmetrical film arrangement" refers to film materials wherein sensitivity, gradation and/or spectral sensitivity is equal or not at opposite sides of the film support. Further the term "symmetrical or asymmetrical pair of screens" refers to screens wherein speed and/or spectral sensitivity is equal or not for both screens.

The photographic material containing spectrally sensitized tabular grains used in the system according to the present invention is image-wise exposed to visible light, preferably green light, generated from converted X-rays emitted by an X-ray source emitting X-rays with an energy adapted to the specific application. Conversion of X-rays proceeds by the preferred green light-emitting phosphors making part of the screens of the image forming film-screen system according to this invention.

Of course processing conditions and composition of processing solutions after image-wise exposure of the film material for use in the system according to this invention are dependent from the specific type of photographic material in which the spectrally sensitized tabular grains are applied. For example, in a preferred embodiment of materials for X-ray diagnostic purposes said materials are adapted to rapid processing conditions. Preferably an automatically operating processing apparatus is used provided with a system for automatic regeneration of the processing solutions. The forehardened material may be processed using one-part package chemistry or three-part package chemistry. Applications within total processing times of 30 seconds and even shorter up to processing times of 120 seconds, known as common praxis, are possible. From an ecological point of view it is even possible to use sodium thiosulphate instead of ammonium thiosulphate in the fixer solution. Useful processing compositions in the processing of films used in the system according to this invention have been described in EP-A 0 542 354, which is incorporated herein by reference.

The following examples illustrate the invention without however limiting it thereto.

## EXAMPLES

### 1. Blue Colored Dyes: Trade Names and Structural Formulas

| DYE | MARKETED BY | TRADE NAME             |
|-----|-------------|------------------------|
| A   | ICI         | Lutetia cyanine ENJPDR |
| B   | BASF        | Paligenblau D6470      |
| C   | Bayer       | Macrolexblau RR        |

-continued

| DYE | MARKETED BY | TRADE NAME       |
|-----|-------------|------------------|
| D   | Hoechst AG  | Reflex Blue 3G51 |
| E   | Hoechst AG  | Reflex Blue R54  |

### 2. Solubility of Blue Dyes

The solubility in mg/l (milligrams per liter) of dyes A-E was determined in water and in isopropanol (SOLIP=solubility in isopropanol) at 25° C. by absorption spectroscopy. The accuracy with which said solubility was measured is about 10 mg/l.

| DYE | SOLUBILITY |             |
|-----|------------|-------------|
|     | water      | isopropanol |
| A   | <10 mg/l   | <10 mg/l    |
| B   | <10 mg/l   | <10 mg/l    |
| C   | <10 mg/l   | 340 mg/l    |
| D   | <10 mg/l   | 175 mg/l    |
| E   | 175 mg/l   | 175 mg/l    |

### 3. Preparation of the Dispersions of the Blue Colored Dyes

20 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 918

A tabular silver bromoiodide emulsion, containing 1 mole % of AgI and 99 mole % of AgBr, was precipitated using the double jet technique. The excessive amount of soluble  $\text{KNO}_3$  salt generated during precipitation of AgBr(I) crystals was removed by washing after emulsion flocculation following said precipitation. The crystals of the thus obtained tabular grain emulsion, containing 75 grams of gelatin per mole of  $\text{AgNO}_3$ , had the following characteristics tics, determined according to the method described in U.S. Pat. No. 4,414,304:

mean diameter of a circle with the same projective surface of the tabular grain:  $1.124 \pm 0.23 \mu\text{m}$  (0.23 being the standard deviation s).

mean thickness of the tabular grains:  $0.23 \mu\text{m}$ .

aspect-ratio: 5.5.

procentual part of the total projective surface of all grains present, covered by the tabular grains: 98%.

#### 4.3.2. Chemical sensitization

This emulsion was chemically sensitized in the presence of anhydro-5,5'-dichloro-3,3'-bis(n.sulfobutyl)-9-ethyloxacarbocyanine hydroxide, chloro auric acid, sodium thiosulphate and potassium thiocyanate.

#### 4.3.3. Preparation of the coating solution of the emulsion layer.

Per mole of  $\text{AgNO}_3$  were added to the above described emulsion at  $40^\circ\text{C}$ : 0.29 g of 4-hydroxy-6-methyl-1,3,3a,7-tetra-azaindene; 9.1 g of sorbitol; 14.5 g of poly ethyl acrylate (MW=1000000); 3.05 g of 1,3-dihydroxybenzene; 31 g of dextrane (MW=10000); 10 g of gelatin and demineralized water in an amount necessary to get an appropriate wet coating thickness.

#### 4.4. Preparation of the coating solution of the intermediate layer.

To 800 ml of demineralized water were added: 44 g of gelatin and 44 g of a solution, 30% by weight, of KIESELSOL 300F (trademarked product from Bayer AG, Leverkusen, Germany). Demineralized water was added to obtain the appropriate wet coating thickness and the desired amount of gelatin per  $\text{m}^2$ .

#### 4.5. Preparation of the coating solution of the protective layer 1.

To 800 ml of demineralized water were added: 44 g of gelatin; 44 g of a solution (30% by weight) of KIESELSOL 300F (trademarked by BAYER AG), 0.92 g of polymethylmethacrylate (average particle diameter:  $3.5 \mu\text{m}$ ); 0.3 g of ammoniumperfluorocaprylate and 10.8 g of a solution (37% by weight) of formaldehyde.

Demineralized water was added to obtain the appropriate wet coating thickness and the desired amount of gelatin per  $\text{m}^2$ .

#### 4.6. Preparation of the coating solution of the protective layer 2.

To 800 ml of demineralized water were added: 44 g of gelatin; 44 g of a solution (30% by weight) of KIESELSOL 300F, 1.84 g of poly methyl methacrylate (average particle diameter:  $3.5 \mu\text{m}$ ); 0.6 g of ammoniumperfluorocaprylate and 21.6 g of a solution (37% by weight) of formaldehyde. Demineralized water was added to obtain the appropriate wet coating thickness and the desired amount of gelatin per  $\text{m}^2$ .

#### 4.7. Coating method of the photographic materials

The materials were obtained by coating at  $38^\circ\text{C}$ , on the support provided with a subbing layer at both sides, the above described coating solutions for the emulsion layer, the intermediate and/or the protective (outermost antistress) layer respectively. Said materials were dried under controlled conditions of humidity and temperature, said tem-

perature never exceeding  $30^\circ\text{C}$ . The emulsion layer, intermediate layer (if present) and protective layer were coated simultaneously by the slide hopper coating technique with the emulsion layer in direct contact with the subbing layer, the intermediate layer thereupon and as an outermost layer of the material the protective (antistress) layer. Before drying the thickness (known as "wet thickness") of the emulsion layer was  $44 \mu\text{m}$ . Per  $\text{m}^2$  and per side of the support the emulsion layer contained an amount of 3.8 g of AgBr(I), said amount being expressed as the equivalent amount of silver nitrate, and of 1.9 g of gelatin. The wet coating thickness and the gelatin content per  $\text{m}^2$  of the protective and intermediate layers are given hereinafter in the description of the material compositions.

#### 5. Evaluation Procedures

##### 5.1. Determination of photographic sensitivity

Samples of the photographic materials were exposed using a continuous wedge with green light of 540 nm during 0.1 seconds and were processed in a 45 seconds cycle of a CURIX HT530 (Agfa-Gevaert trademarked name) processor.

Commercially available G138 developer and G334 fixer, both trademarked names from Agfa-Gevaert, were used as processing chemicals.

The density as a function of the light dose ( $\log E$ ) was then measured and the  $\log E$  value at a density of 1.00 above fog was determined. This value was representing the sensitivity of the material. A more sensitive material has a lower  $\log E$  value (requires a lower light dose).

##### 5.2. Determination of fog

Unexposed samples were processed in the above described processing cycle. The specular density for white light was then determined. This fog thus includes the density of the blue dyes in the undercoat layer (support) and in the layers coated thereupon.

##### 5.3. Determination of $L$ , $a^*$ , $b^*$ of developed Ag

Samples of the materials were exposed in order to obtain the maximum density and were processed in the above described processing cycle. The color of the developed Ag, viewed by incident light was measured as CIELAB values:  $L$ ,  $a^*$ ,  $b^*$ .

Therefor a GRETAG spectrophotometer was used with  $45^\circ/0^\circ$  measuring geometry,  $20^\circ$  standard observer and standard illuminant D65.

##### 5.4. Determination of dye stain at the surface of the X-ray screen

The X-ray screen (format 24 cm $\times$ 30 cm) was made slightly wet with Agfa-Gevaert Curix "screen-cleaner". This screen-cleaner mainly consists of isopropanol.

On the wetted X-ray screen, samples of the undeveloped photographic materials were placed. Thereupon a cardboard and a weight of 10 kg was placed during 2 hours.

The samples were then removed and the color of the X-ray screen was examined for appearance of dye stain. When dye stain was present, this X-ray screen was treated to be cleaned with the Curix "screen-cleaner". When the dye stain disappeared, the dye stain was called "cleanable".

The X-ray screen used in this dye stain test was CURIX ORTHO REGULAR 1FFJ5P (trademarked screen by Agfa-Gevaert NV).

##### 5.5. Contamination of the rollers of the Processing machine

800 sheets (format 14"  $\times$  17") were processed in the above described processing cycle. The rollers of the racks of the fixer, of the rinsing and of the drying section were investigated for contamination and dye stain.

#### EXAMPLE 1

Example 1 shows the importance of the location of the blue colored dyes in the material. Therefore materials Nos. 1 to 4 were coated as follows:

## 11

## Material No. 1 (comparison)

Material No. 1 was obtained by coating support 1 as described above with the coating solution of protective layer 1, coated at a wet thickness of 25  $\mu\text{m}$  and at a gelatin content per  $\text{m}^2$  and per side of the support of 1.1 g. No intermediate layer was coated.

## Material No. 2 (comparison)

Material No. 2 was coated just as Material No. 1, except for the use of support 2 instead of support 1 as a support and for the addition of 4.1 g of a dispersion of dye A to the coating solution of the emulsion layer. The coated material contained 9.2  $\text{mg}/\text{m}^2$  and per side of dye A in the emulsion layer.

## Material No. 3 (comparison)

Material No. 3 was coated as Material No. 2, except for the addition of 3.7 g of a dispersion of dye A which was added to the coating solution of the protective layer 1. This material thus contained 9.2  $\text{mg}/\text{m}^2$  and per side of dye A in the protective layer.

## Material No. 4 (invention)

Material No. 4 comprises an intermediate layer coated at a wet thickness of 12.5  $\mu\text{m}$ . Adjacent thereto and farther from the support the protective layer 2 was coated, also at a wet thickness of 12.5  $\mu\text{m}$ . The gelatin content per  $\text{m}^2$  of the intermediate and the protective layer was 0.55 g for both. An amount of 7.4 grams of a dispersion of dye A was added to the coating solution of the intermediate layer. This material thus contained 9.2  $\text{mg}/\text{m}^2$  and per side of dye A, said dye being located in the intermediate layer.

In Table I for the materials Nos. 1 to 4, No. 4 being coated according to this invention, data are summarized about  $\text{La}^* \text{b}^*$ -values, reflecting the color of the developed silver, together with values of fog (FOG), photographic sensitivity, presence (YES) or absence (NO) of a contamination of the rollers of the processing machine.

TABLE I

| MATL | dye location       | Sensit. |      |       | contamination rollers | 30                       |
|------|--------------------|---------|------|-------|-----------------------|--------------------------|
|      |                    | FOG     | logE | L     |                       |                          |
| 1    | No dye             | 0.173   | 1.75 | 17.30 | 1.77                  | 4.14 NO                  |
| 2    | emulsion layer     | 0.171   | 1.95 | 16.89 | 1.62                  | 4.01 NO                  |
| 3    | protective layer   | 0.167   | 1.73 | 16.86 | 0.73                  | 2.78 YES, blue dye stain |
| 4    | intermediate layer | 0.168   | 1.73 | 16.87 | 0.75                  | 2.76 NO                  |

From Table I it can be concluded that addition of the dispersion of dye A to the protective layer or to the intermediate layer results in a more neutral (black) image tone (lower value of  $\text{b}^*$ ) of developed silver without loss of the photographic speed or increase of the fog level. However addition of dye A to the protective layer results in an unwanted blue stain on the rollers of the fixer rack, which is not the case for the material of the invention (No. 4) wherein dye A is added to the intermediate layer.

## EXAMPLE 2

Example 2 shows the necessity to use blue dyes having a low solubility in isopropanol. Therefore Materials Nos. 5 to 8 were additionally coated:

Material No. 5 was coated just as Material No. 4 except for the use of 10.8 g of a dispersion of dye B instead of dye A which was added to the coating solution of the intermediate layer. This material then contained 13.5  $\text{mg}/\text{m}^2$  of dye B per side of the support.

## 12

Material No. 6 was coated just as Material No. 4 except for the addition of 14.5 grams of a dispersion of dye C instead of dye A which was added to the coating solution of the intermediate layer. This material then contained 18.7  $\text{mg}/\text{m}^2$  of dye C per side of the support.

Material No. 7 was coated just as Material No. 4 except for the addition of 4.6 grams of a dispersion of dye D instead of dye A which was added to the coating solution of the intermediate layer. This material then contained 5.8  $\text{mg}/\text{m}^2$  of dye D per side of the support.

Material No. 8 was coated just as Material No. 4 except for the addition of 4.9 grams of a dispersion of dye E instead of dye A which was added to the coating solution of the intermediate layer. This material then contained 6.1  $\text{mg}/\text{m}^2$  of dye E per side of the support.

In Table II for the Materials Nos. 1 and 4-8 which were coated as described hereinbefore data are summarized about  $\text{La}^* \text{b}^*$ -values, reflecting the color of the developed silver, together with values of fog (FOG), coated amount of dye (DYE) in the intermediate layer and with data for the solubility in isopropanol (SOLIP), expressed in mg/l, of the corresponding dye.

Materials Nos. 4 and 5 were coated according to this invention.

TABLE II

| MATL                    | DYE | SOLIP (mg/l) | FOG   | L     | a*   | b*   | Screen stain |
|-------------------------|-----|--------------|-------|-------|------|------|--------------|
| 1<br>(comparison)       | —   | —            | 0.173 | 17.30 | 1.77 | 4.14 | No           |
| 4<br>(invention)        | A   | <10          | 0.168 | 16.87 | 0.75 | 2.76 | No           |
| 5<br>(invention)        | B   | <10          | 0.172 | 16.45 | 1.41 | 3.24 | No           |
| 35<br>6<br>(comparison) | C   | 340          | 0.172 | 16.44 | 1.11 | 2.91 | Yes**        |
| 7<br>(comparison)       | D   | 175          | 0.172 | 16.41 | 0.84 | 3.02 | Yes**        |
| 8<br>(comparison)       | E   | 175          | 0.180 | 16.70 | 1.18 | 2.74 | Yes**        |

\*\*not cleanable X-ray screen

As can be concluded from Table II the addition of a dispersion of a blue dye to the intermediate layer results in a more neutral (black) image tone (lower value of  $\text{b}^*$ ) of the developed silver, generated from tabular grain emulsions, after examination of said developed silver under reflected light conditions.

Further comparative materials coated from dyes, showing a high solubility in isopropanol, are characterized by an unremovable dye staining of the screens held in contact therewith, whereas materials having a composition according to this invention and thus coated with dyes showing a low solubility in isopropanol, are characterized by the absence of dye staining at the surface of intensifying screens.

I claim:

1. Image forming film-screen system for medical diagnostic imaging comprising a light-sensitive silver halide photographic film material in operative association with at least one intensifying screen comprising on a support a layer of a visible light emitting luminescent phosphor, the said film material comprising a support and on at least one side thereof a light-sensitive silver halide emulsion layer having spectrally sensitized tabular silver halide and a non-light-sensitive protective layer, wherein said protective layer contains a polymeric compound selected from the group

**13**

consisting of gelatin, a synthetic, semi-synthetic or natural substitute for gelatin and latex (co)polymers, in an amount of at least 0.4 g per m<sup>2</sup>; characterized in that between a light-sensitive silver halide emulsion layer and said protective layer on the same side of the support as the said protective layer there is an intermediate layer comprising a blue colored pigment in dispersed form, having a solubility in isopropanol at 25° C. of less than 10 mg per liter.

2. System according to claim 1, wherein said blue colored pigment in dispersed form has a maximum absorption in the visible wavelength region from 570 to 700 nm.

3. System according to claim 1, wherein said blue colored pigment in dispersed form has a maximum absorption in the visible wavelength region from 570 to 630 nm.

4. System according to claim 1, wherein said blue colored pigment is a pigment or dye selected from the group consisting of phthalocyanine dyes and indanthron dyes.

5. System according to claim 1, wherein said blue pigment is present in said intermediate layer in an amount of from 1 mg/m<sup>2</sup> to 100 mg/m<sup>2</sup>.

**14**

6. System according to claim 1, wherein an average mean particle size of said blue colored pigment in dispersed form is not more than 0.5  $\mu\text{m}$ .

7. System according to claim 1, wherein said light-sensitive tabular silver halide grains have an aspect ratio of from 2 to 20, a thickness from 0.06 to 0.30  $\mu\text{m}$  and account for at least 50% of the total projective area of all grains and are spectrally sensitized to the green region of the wavelength spectrum.

8. System according to claim 1, wherein said screen is an intensifying screen comprising at least one green light-emitting luminescent phosphor.

9. System according to claim 8, wherein said green light-emitting luminescent phosphor is a Gd<sub>2</sub>O<sub>2</sub>S:Tb phosphor.

10. Light-sensitive silver halide photographic film material as defined in claim 1.

\* \* \* \* \*